

# United States Patent Office

2,735,048

Patented Feb. 14, 1956

1

2,735,048

## POWER TRANSMISSION DEVICE

Moerue D. Levy, University City, Mo., assignor to Vickers Incorporated, Detroit, Mich., a corporation of Michigan

No Drawing. Application March 15, 1951,  
Serial No. 215,867

14 Claims. (Cl. 317—234)

This invention relates to power transmission and more particularly to blocking layer devices such as selenium rectifier and light-sensitive cells, and to methods of making such devices.

In the manufacture of blocking layer devices, such as selenium rectifiers, the following steps are generally observed: (1) a layer of amorphous selenium is applied to a conductive base such as nickel-coated iron, aluminum, etc.; (2) the selenium layer is heat-treated to change it from the amorphous state to its conducting crystalline form; (3) an "artificial" barrier layer, such as lacquer, may or may not be applied to the selenium surface to affect the characteristics of the final product; (4) a counterelectrode of low melting point alloy is applied to the selenium surface by some suitable method such as spraying; and (5) the completed cell undergoes an electroforming process to increase the rectification ratio.

Rectification is generally believed to occur at the interface of the counterelectrode and the selenium layer, due to a barrier at that point. The nature of this barrier is not known with any degree of certainty. Heretofore, many "artificial" barriers have been proposed and used. These are generally formed by treating the annealed selenium layer with one or another agent or agents before the application of the counterelectrode. Many such agents have been employed with varying degrees of success in improving the rectification ratio of rectifier cells.

The present invention has special utility in the manufacture of selenium rectifier cells and improving the rectification ratio thereof, and involves the use of quaternary ammonium hydroxides as barrier forming agents which are applied to the annealed selenium surface after which the counterelectrode is processed, and the integral unit is then baked at suitable temperatures until the reaction product at the selenium and counterelectrode interface reaches a state providing the desired rectification ratio in the end product. After the baking step the unit is electroformed in the usual manner.

It is therefore an object of the invention to provide a method of forming an artificial barrier layer in a blocking layer device.

Another object of the invention is to provide a method of making a blocking layer device with improved rectification characteristics.

Still another object of the invention is to provide a blocking layer device having improved electrical characteristics.

Further objects and advantages of the present invention will be apparent from the following description.

In accordance with the invention herein, a conductive base plate, for example, nickel-coated iron, is coated with amorphous selenium by any suitable method after which the selenium is annealed to change it into its crystalline or conducting state. Next, a suitable quantity of a quaternary ammonium hydroxide with groups having three carbon atoms or less in the chains, for example, tetraethanol ammonium hydroxide, is uniformly applied to the annealed selenium surface, preferably by spraying a solution of the hydroxide in a suitable solvent. For manufacturing convenience, quick drying solvents are

preferred, such as low boiling point alcohols, low boiling point ketones, etc. Examples of such solvents are methyl alcohol, ethyl alcohol, isopropyl alcohol, acetone, and ethyl methyl ketones. Water may be used as a solvent with a sacrifice in the uniformity of the applied coating because of low wetting ability.

Although the selenium coated plates may be dipped in the solution, spraying permits a better control of the concentration per unit area. The actual amount of the hydroxide required on the plates is dependent upon the cell characteristics desired, and is best determined empirically. An increase in concentration decreases the reverse conductivity of the cell, and to a much lesser extent the forward conductivity of the cell. Thus, the rectification ratio is improved with any increase in concentration. However, too great a concentration will result in an impractical low forward conductivity even though the resulting rectification ratio in itself will be high.

The degree of concentration of the hydroxide in the solvents is governed by factors such as the amount per unit area desired after the evaporation of the solvents, and the method of application. In spraying, the type of nozzle, the spray velocity, the speed of the plates passing under the nozzle, and the number of passes are factors which enters into the determination of the ratio of the hydroxide concentrate in the solvents.

In general, concentrations on a volume basis of about one part of the hydroxide in 50 to 1000 parts of solvent provides a wide variety of concentrations from which a suitable choice may be made in connection with any selected method of application.

With the fast drying solvent the sprayed solution dries almost as fast as it hits the selenium surface.

The method herein may be practiced with any of the quaternary ammonium hydroxides having groups with three carbon atoms or less in the chains, i. e., having the general formula:



where N is the nitrogen atom, OH is the hydroxyl radical, and each R is a radical or group having three carbon atoms or less, for example, tetraethanol ammonium hydroxide whose formula is



Other examples of such hydroxides are: tetramethyl ammonium hydroxide



tetraethyl ammonium hydroxide



tetrapropynol ammonium hydroxide



The general formula



is intended to cover not only the case where each R is the same, but also where the radicals are mixed, for example, dimethyl diethyl ammonium hydroxide



It is apparent that each R is a radical having three carbon atoms or less.

After the hydroxide application is dry, a suitable counterelectrode is placed on the treated selenium surface. For instance, the counterelectrode may be formed by spraying onto the treated selenium surface a low melting metal or alloy. There are many known alloys usable as counterelectrodes and the process herein is not confined to the use of any particular counterelectrode material. Examples of commonly used alloys which were used in the practice of the method herein are: 70% tin-30% cadmium; 20% tin-80% cadmium; and the 130° eutectic alloy of tin, bismuth, and cadmium.

After the counterelectrode is applied the composite unit is heated by any suitable means such as baking in an oven. The heating temperature is preferably below the melting point of the electrodes, and the temperature and the length of heating time may be varied depending upon the final cell characteristics desired.

Although the temperature and time of heating or baking is not critical, the most practical ranges extend from about 50° C. to about 150° C., and from about ten minutes to about six hours. The lower the temperature, the more time is required to achieve a particular end characteristic. Tests show that for a selected temperature the end characteristic will vary with the heating time. In a test of a series of cells made according to the method herein and where the melting point of the counterelectrode was 103°, a baking temperature of 95° was selected, and the following results were tabulated after the cells were electroformed.

The following tables show examples of cell groups treated by spraying the crystalline layers with tetraethanol ammonium hydroxide in intermediate concentrations by volume of one part hydroxide in 250, 500, and 750 parts methyl alcohol, respectively.

## Concentration 1 part in 750

| No. of Cells | Time of Baking @ 95° C., minutes | Av. Voltage |         | Rect. Ratio |
|--------------|----------------------------------|-------------|---------|-------------|
|              |                                  | Inverse     | Forward |             |
| 10.          | 20                               | 27.3        | 1.09    | 26.0        |
| 10.          | 60                               | 24.1        | 1.07    | 22.5        |
| 10.          | 120                              | 26.2        | 1.01    | 26.0        |
| 10.          | 240                              | 25.0        | 1.06    | 23.6        |

## SAME CELLS AFTER 1 WEEK SHELF AGING

|     | 20  | 29.7 | 1.39 | 21.4 |
|-----|-----|------|------|------|
| 10. | 60  | 26.4 | 1.06 | 24.9 |
| 10. | 120 | 26.8 | 1.05 | 25.5 |
| 10. | 240 | 26.1 | 1.06 | 24.6 |

## Concentration 1 part in 500

| No. of Cells | Time of Baking @ 95° C., minutes | Av. Voltage |         | Rect. Ratio |
|--------------|----------------------------------|-------------|---------|-------------|
|              |                                  | Inverse     | Forward |             |
| 10.          | 20                               | 28.5        | .98     | 29.1        |
| 10.          | 60                               | 26.2        | .99     | 25.5        |
| 10.          | 120                              | 27.5        | 1.08    | 25.4        |
| 10.          | 240                              | 27.9        | 1.11    | 25.1        |

## SAME CELLS AFTER 1 WEEK SHELF AGING

|     | 20  | 30.4 | 1.20 | 23.5 |
|-----|-----|------|------|------|
| 10. | 60  | 29.1 | 1.17 | 24.8 |
| 10. | 120 | 28.6 | 1.17 | 24.4 |
| 10. | 240 | 30.4 | 1.18 | 25.7 |

4  
Concentration 1 part in 250

| No. of Cells | Time of Baking @ 95° C., minutes | Av. Voltage |         | Rect. Ratio |
|--------------|----------------------------------|-------------|---------|-------------|
|              |                                  | Inverse     | Forward |             |
| 10.          | 20                               | 35.9        | 1.06    | 34.0        |
| 10.          | 60                               | 32.6        | 1.06    | 30.7        |
| 10.          | 120                              | 35.7        | 1.37    | 26.0        |
| 10.          | 240                              | 32.6        | 1.12    | 29.1        |

## SAME CELLS AFTER 1 WEEK SHELF AGING

|     | 20  | 37.8 | 1.66 | 22.7 |
|-----|-----|------|------|------|
| 10. | 60  | 35.4 | 1.49 | 23.7 |
| 10. | 120 | 36.9 | 1.53 | 24.1 |
| 10. | 240 | 35.1 | 1.3  | 27.0 |

The above charts indicate that higher concentrations decrease the reverse conductivity and that cell stability is enhanced by a longer heating time. The charts also indicate that with a longer baking time, shelf aging after electroformation tends to further improve the rectification ratio. It is preferable to stabilize the plates by aging them after electroformation, regardless of the baking time employed.

Improvements of at least 24% in the rectification ratio of the end product have been obtained by the addition of the baking step.

After the baking step, the composite unit is electroformed by any suitable method, such as applying unidirectional current to the cell in the reverse direction until the desired rectification ratio is attained.

The term "baking" as used throughout the specification and claims is intended to cover all forms of heating.

While the form of embodiment of the invention as herein disclosed constitutes a preferred form, it is to be understood that other forms might be adopted, all coming within the scope of the claims which follow.

What is claimed is as follows:

1. A method of forming a barrier layer in a selenium blocking layer cell which comprises surface treating a crystalline selenium layer with a quaternary ammonium hydroxide, applying a counterelectrode to the treated selenium surface, baking the composite cell before any electroforming, and electroforming the cell, and quaternary ammonium hydroxide having the general formula



where each R is a group having less than four carbon atoms.

2. The method of producing blocking layer devices which comprises providing a supporting base with a layer of crystalline selenium, applying a quaternary ammonium hydroxide to the surface of the selenium, applying a counterelectrode to the treated selenium surface, and baking the composite product, said quaternary ammonium hydroxide having the general formula



where each R is a group having less than four carbon atoms.

3. A method of making blocking layer devices having a crystalline selenium layer on a base which comprises the steps of applying to the crystalline selenium surface a solution of a quaternary ammonium hydroxide in a solvent, applying a counterelectrode to the treated selenium surface, baking the composite product before any electroforming, and electroforming the device said quaternary ammonium hydroxide having the general formula



where each R is a group having less than four carbon atoms.

4. A method of making blocking layer devices having a crystalline selenium layer on a base which comprises the steps of applying to the crystalline selenium surface a solution of a quaternary ammonium hydroxide in a solvent, applying a counterelectrode to the treated selenium surface, baking the composite product before any electroforming, and electroforming the device, the concentration range of the quaternary ammonium hydroxide being about one part by volume in from 50 to 1000 parts of solvent, said quaternary ammonium hydroxide having the general formula



15

where each R is a group having less than four carbon atoms.

5. A method for forming a barrier layer in a selenium blocking layer device which comprises surface treating a crystalline selenium layer with a solution of a quaternary ammonium hydroxide in a solvent, applying a counterelectrode to the treated selenium surface and baking the composite product, said quaternary ammonium hydroxide having the general formula



30

where each R is a group having less than four carbon atoms.

6. A method for forming a barrier layer in a selenium blocking layer device which comprises surface treating a crystalline selenium layer with a solution of a quaternary ammonium hydroxide in a solvent, and baking the composite product, the concentration range of the quaternary ammonium hydroxide being about one part by volume in from 50 to 1000 parts of solvent, said quaternary ammonium hydroxide having the general formula



where each R is a group having less than four carbon atoms.

7. A method of making blocking layer devices having a crystalline selenium layer on a base which comprises the steps of applying tetraethanol ammonium hydroxide to the crystalline selenium surface, applying a counterelectrode to the treated selenium surface, baking the composite product before any electroforming, and electroforming the device.

8. A method of making blocking layer devices having a crystalline selenium layer on a base which comprises the steps of applying tetraethanol ammonium hydroxide in a solvent to the crystalline selenium surface, applying a counterelectrode to the treated selenium surface, baking the composite product before any electroforming, and electroforming the device, the concentration range of the tetraethanol ammonium hydroxide being about one part by volume in from 50 to 1000 parts of solvent.

9. A method for forming a barrier layer in a selenium blocking layer device which comprises surface treating a crystalline selenium layer with tetraethanol ammonium hydroxide, applying a counterelectrode to the treated selenium surface and baking the composite product.

10. A method for forming a barrier layer in a selenium blocking layer device which comprises surface treating a crystalline selenium layer with tetraethanol ammonium

hydroxide in a solvent, applying a counterelectrode to the treated selenium surface, and baking the composite product, the concentration range of the tetraethanol ammonium hydroxide being about one part by volume in from 50 to 1000 parts of solvent.

11. A blocking layer device comprising a crystalline selenium layer, a counterelectrode on said layer, and a barrier layer between the electrode and the selenium layer, said barrier being the product formed by the interposition of a quaternary ammonium hydroxide between the electrode and the selenium surface and baking the composite unit before any electroforming, said quaternary ammonium hydroxide having the general formula



6

where each R is a group having less than four carbon atoms.

12. A blocking layer device comprising a conductive base, a layer of crystalline selenium on the base, the surface of the selenium being treated with a quaternary ammonium hydroxide, and a counterelectrode on the treated selenium surface, the composite device being baked, said quaternary ammonium hydroxide having the general formula



30

where each R is a group having less than four carbon atoms.

13. A blocking layer device comprising a conductive base, a layer of crystalline selenium on the base, the surface of the selenium being treated with a quaternary ammonium hydroxide, a counterelectrode on the treated selenium surface, and a barrier layer between the electrode and the surface of the selenium, the barrier layer being the product resulting from the reaction of the quaternary ammonium hydroxide due to baking of the composite unit before any electroforming.

14. A blocking layer device comprising a conductive base, a layer of crystalline selenium on the base, the surface of the selenium being treated with a quaternary ammonium hydroxide, a counterelectrode on the treated selenium surface, and a barrier layer between the electrode and the surface of the selenium, the barrier layer being the product resulting from the reaction of the quaternary ammonium hydroxide due to baking of the composite unit, said quaternary ammonium hydroxide having the general formula



where each R is a group having less than four carbon atoms.

References Cited in the file of this patent

UNITED STATES PATENTS

|           |                |               |
|-----------|----------------|---------------|
| 2,255,358 | Jackson et al. | Sept. 9, 1941 |
| 2,362,545 | Ellis et al.   | Nov. 14, 1944 |
| 2,395,259 | Ellis et al.   | Feb. 19, 1946 |
| 2,471,898 | Rau            | May 31, 1949  |
| 2,507,782 | Goodman        | May 16, 1950  |

FOREIGN PATENTS

|         |           |               |
|---------|-----------|---------------|
| 125,065 | Australia | Apr. 29, 1944 |
|---------|-----------|---------------|